

1

2,789,951

## COMPOUNDED TURBINE OILS

Raymond T. Kern, Jr., Allentown, Pa., and John G. Peters, Audubon, N. J., assignors to Gulf Oil Corporation, Pittsburgh, Pa., a corporation of Pennsylvania

No Drawing. Application August 19, 1954,  
Serial No. 451,039

8 Claims. (Cl. 252—32.7)

This invention relates to lubricating compositions and more particularly to compounded turbine oils adapted to prevent rusting and corrosion of metal turbine parts which are exposed to moisture.

Various lubricating compositions have heretofore been disclosed for lubricating steam turbines but the prior compositions have not been entirely satisfactory. Some of the prior compositions have exhibited good resistance to oxidation but they have not given complete protection against rusting and corrosion of metal turbine parts which are exposed to moisture. Other compositions have given good protection against rusting and corrosion in the presence of moisture, but the moisture has given rise to the formation of an undesirable precipitate.

The present invention is based upon a particularly effective lubricating composition having good resistance to oxidation combined with good lubricating characteristics and corrosion and rust-inhibiting properties with the added advantage that no precipitate is formed when the composition becomes contaminated with water.

The improved lubricating composition of this invention consists essentially of a homogeneous mixture of lubricating oil, a metal alkyl thiophosphate, an alkyl phenol, a substantially neutral addition product of isoamyl octyl acid phosphate with primary fatty amines containing from 8 to 18 carbon atoms, and an acid ester of (1) a dimeric acid derived from an unsaturated fatty acid containing from 6 to 22 carbon atoms and having from 2 to 3 ethylenic linkages per molecule and (2) a partial ester of a fatty acid containing from 12 to 24 carbon atoms and an alkitol anhydride. An improved lubricating composition can be prepared by incorporating in an oil a metal alkyl thiophosphate, an alkyl phenol and a substantially neutral addition product of isoamyl octyl acid phosphate with primary fatty amines containing from 8 to 18 carbon atoms. While the composition thus obtained has good corrosion and rust-inhibiting properties, the composition has a disadvantage in that it forms a precipitate when contaminated with water.

We do not wish to be limited to any theory with respect to the reason that a precipitate is formed when a small amount of water contaminates the composition containing no acid ester. However, it appears that the metal alkyl thiophosphate and the fatty amine salt of isoamyl octyl acid phosphate are incompatible in the presence of moisture and that they react to form a material which settles out of solution. This settling out is undesirable in that useful constituents are removed from the lubricating oil thus cutting down on its effectiveness. In addition to affecting the usefulness of the composition, its appearance is impaired as it becomes cloudy and is heterogeneous instead of being homogeneous.

We have found that these undesirable properties can be overcome by incorporating in the composition a small amount of an acid ester of (1) a dimeric acid derived from an unsaturated fatty acid containing from 6 to 22 carbon atoms and having from 2 to 3 ethylenic linkages

2

per molecule and (2) a partial ester of a fatty acid containing from 12 to 24 carbon atoms and an alkitol anhydride.

The lubricating oil to which the other constituents are added is advantageously a highly refined paraffinic oil. By the term "highly refined paraffinic oil" we mean a petroleum lubricating oil which has been refined by one of the more drastic refining methods known in the art, for example, by conventional aluminum chloride refining or by a solvent extraction adapted to remove all or substantially all of the unsaturated and naphthenic constituents of the oil. Aluminum chloride refined or solvent extracted paraffinic base oil, such as a Pennsylvania oil, provides an excellent base oil for the composition of the invention. However, drastically refined Mid-Continent and Gulf Coastal oil may also be used.

The metal alkyl thiophosphates which can be used in accordance with the invention are advantageously those whose metal component is a metal of group II of Mendeleff's periodic arrangement of the elements. Included within this group are magnesium, calcium, zinc, strontium, cadmium and barium. However, other metals including aluminum, copper, lead, tin, iron and manganese can also be employed. The alkyl constituents are preferably those containing between 3 and 12 carbon atoms. Examples of the alkyl groups which can be used are butyl, particularly tertiary butyl, amyl, isoamyl, tertiary amyl, hexyl, heptyl, octyl, nonyl, decyl, dodecyl, and the like. While the mono-alkyl esters can be used, the di-alkyl esters are particularly suitable for the purposes of the invention. An example of a particularly effective compound which can be used is zinc dihexyl thiophosphate. When zinc dihexyl thiophosphate is used, it is preferably used in an amount between about 0.01 and 0.1 percent by weight based on the weight of the total composition. An amount greater than about 0.1 percent is undesirable in that the neutralization number of the final product is increased above the maximum set for commercial use.

The alkyl phenol which is used in accordance with the invention is advantageously a di- or tri-alkylated phenol or cresol with at least one of the alkyl groups being a tertiary alkyl group. The alkyl groups are preferably those containing between 3 and 12 carbon atoms. Good results can be obtained with a tri-tertiary butyl phenol or a di-tertiary butyl cresol. Examples of the preferred alkylated phenols are 2,4,6-tri-tertiary-butylphenol, 2,6-di-tertiary-butyl-4-methylphenol and bis(2-hydroxy-3-tertiary-butyl-5-methylphenyl)methane. The alkyl phenols are advantageously used in amounts of about 0.1 to about 2.0 percent by weight based on the weight of the total composition.

The fatty amine salt of isoamyl octyl acid phosphate which can be used in accordance with the invention is prepared by reacting isoamyl octyl acid phosphate with a primary fatty amine containing from 8 to 18 carbon atoms. One example of a primary fatty amine suitable for the purpose of this invention is cocoamine, which is a commercially available product prepared by converting coconut oil fatty acids into the corresponding amine. It consists mostly of monolauryl amine with minor amounts of adjacent homologues. The cocoamine salt of isoamyl octyl acid phosphate and its preparation are fully described in U. S. Patent No. 2,371,851 which issued on March 20, 1945, to Herschel G. Smith and Troy L. Cantrell. As disclosed in said patent, the cocoamine salt of isoamyl octyl acid phosphate can be readily prepared by reacting cocoamine with isoamyl octyl acid phosphate in approximately equimolecular ratios, the reaction being so controlled as to produce substantially neutral reaction mixtures having a pH value within the range 5.5 to 7.5, as illustrated in Examples 1 and 2 of that patent. The isoamyl octyl acid

phosphate employed is a di-ester of orthophosphoric acid having the following formula:



This compound is also known as 3-methylbutyl,2-ethyl-hexyl acid orthophosphate. It readily reacts with cocoamine and other primary fatty amines containing from 8 to 18 carbon atoms. Instead of cocoamine we can use other primary fatty amines containing from 8 to 18 carbon atoms. These amines include mono-capryl,



mono-lauryl, mono-myristyl, mono-palmityl and mono-stearyl amines. The fatty acid amine salt of isoamyl octyl acid phosphate is preferably used in an amount between about 0.005 and about 0.2 percent by weight based on the weight of the total composition.

The acid esters employed in accordance with this invention are the reaction products resulting from the esterification of a dimerized unsaturated fatty acid with a partial fatty acid ester of an alkitol anhydride. The ratio of reactants may range from one mol of dimerized acid per mol of partial fatty acid ester up to the number of mols of dimerized acid that is equal to the number of free hydroxyl groups in the partial fatty acid ester, per mol of partial fatty acid ester.

The esterification reaction is effected in conventional manner and under conventional conditions. Thus, while esterification may proceed slowly at room temperature, the reaction is normally advantageously accelerated by heating the reactants, usually with refluxing, and/or by the use of conventional esterification catalysts, such as hydrogen chloride, sulfuric acid, or an aromatic sulfonic acid, such as p-toluene-sulfonic acid. The reaction may be driven to substantial completion by removing one of the products of reaction. Since the herein disclosed dimeric unsaturated fatty acids, partial esters of alkitol anhydrides, and their reaction products boil at a temperature substantially above the boiling point of water, the reaction conveniently may be driven to completion by removal of the water of esterification by distillation. The removal of water from the reaction mixture may be facilitated by mechanical agitation, or by bubbling an inert gas, such as nitrogen, through the reaction mixture.

By way of illustrating the foregoing process, one, two or three mols of dimerized acid may be esterified with one mol of a partial fatty acid ester containing three free hydroxyl groups, under conventional reaction conditions, with the elimination, respectively, of one, two or three mols of water of esterification, to form, respectively, a mono-, di- or tri-acid or tricarboxylic ester of the dimerized acid and the partial fatty acid ester.

If desired, the reaction products may be prepared by effecting esterification of the reactants in mineral oil solution. This expedient is advantageous in that it prevents localized overheating of the reactants. Moreover, the resulting reaction products are in the form of mineral oil concentrates, the use of which often facilitates solution of the additives in their ultimate vehicles.

The dimerized acids referred to above are dimers, i. e., bimolecular addition products of conjugated or unconjugated dienoic or trienoic fatty acids having from 6 to 22 carbon atoms before dimerization. Dimeric acids derived from dienoic and trienoic fatty acids are well known and can be prepared by conventional methods which form no part of this invention.

More particularly, dimerized acids capable of forming the compounds utilized in the composition of this invention are prepared from dienoic or trienoic fatty acids having the generic formula  $\text{C}_n\text{H}_{2n-x}\text{COOH}$ , where  $n$  is an integer of from 5 to 21 and  $x$  is 3 or 5. As will be evident, such monomeric acids contain from 6 to 22 carbon atoms and may contain 2 or 3 ethylenic linkages as the ratio of carbon to hydrogen increases, i. e., as  $x$  in-

creases from 3 to 5. Dimerized acids corresponding to the addition products of the foregoing acids therefore may be defined by the generic formula:



where  $n$  is an integer of from 10 to 42 and where  $x$  is an even integer of from 6 to 10. These dimeric acids are therefore dibasic or dicarboxylic acids having from 12 to 44 carbon atoms.

Representative members of the class of dimerized acids capable of forming the compounds employed in the compositions of this invention are dimers of dienoic acids such as sorbic (hexadienoic), linoleic (octadecadienoic), humoceric (nonadecadienoic) and eicosinic (eicosadienoic) acids. Dimers of trienoic acids, for example, linolenic and eleostearic (octadecatrienoic) acids also may be used.

It is not necessary that both of the unsaturated fatty acid molecules of the bimolecular addition product be identical. Dimers of mixed composition such as those obtained by dimerizing mixed dienoic, mixed trienoic or mixed dienoic and trienoic acids such as may be derived from certain naturally occurring drying oils, e. g., linseed oil and soybean oil, are quite satisfactory.

Dienoic and trienoic acids having 18 carbon atoms, especially those having conjugated olefinic linkages, are preferred for reasons of economy of procurement, ease of reaction and the general excellence of the additives prepared therefrom.

The partial esters of alkitol anhydrides and fatty acids adapted for use in the formation of the reaction products are those resulting from esterification with the desired fatty acid of at least one, but less than all, of the available hydroxyl groups of an alkitol anhydride. By alkitol anhydride is meant an intramolecular, mono- or di-anhydride of a polyhydric alcohol which contains at least 4 carbon atoms and at least 4 hydroxyl groups, or mixtures of said anhydrides. Representative of the class of alkitals are erythritol; pentitols, such as arabitol, xylitol and adonitol; and hexitols such as mannitol, dulcitol and sorbitol, just as the xylitan and sorbitans are representative of the alkitol anhydrides, or alkitals.

Fatty acids capable of forming partial esters of alkitol anhydrides suited to the preparation of the additives utilized in this invention are the fatty acids containing from 12 to 24 carbon atoms. These acids may be saturated or unsaturated, and they may be substituted with groups which do not adversely affect the oil-solubility or corrosion-inhibiting properties of the final reaction product. Representative of this group of acids are lauric acid, oleic acid, ricinoleic acid, stearic acid and lignostearic acid.

Partial esters capable of reacting to form the reaction products include those formed by reacting a fatty acid of the foregoing kind with the desired alkitol anhydride in a molar ratio of at least 1:1, but less than that which would result in neutralization of all of the hydroxyl groups of the alkitol anhydride. The use of mixtures of partial fatty acid esters of alkitol anhydrides is also included within the scope of the invention. Specific examples of partial esters of alkitol anhydrides capable of reacting with dimeric unsaturated fatty acids to form acid esters which can be used in the composition of the invention are xylitan and sorbitan mono-, sesqui-, di- and tri-oleates and stearates. Partial esters of hexitol anhydrides, i. e., anhydrides of polyhydric alcohols containing 6 carbon atoms and 6 hydroxyl groups, are preferred.

The partial esters of alkitol anhydrides disclosed herein as well as the method of preparing the same are conven-

tional and form no part of the present invention. Accordingly, they need not be described in detail.

Representative specific examples of acid esters of dimeric acids with partial fatty acid esters of alkyls which can be used in the compositions of this invention are the mono- and poly-carboxylic acid esters of dimerized linoleic, linolenic and eleostearic acids with sorbitan and xylitan mono-, sesqui-, di- and trioleates and stearates. Included within the foregoing representative class of compounds are mono-, di-, and tri-acid dilinoleic mono-, di- and tri-esters of sorbitan monooleate, mono- and di-acid dilinoleic mono- and di-esters of sorbitan dioleate, mono-acid dilinoleic mono-esters of sorbitan trioleate, mono- and di-acid dilinoleic mono- and di-esters of xylitan monooleate, mono-acid dilinoleic mono-esters of xylitan dioleate, and corresponding acid esters made from dimerized linolenic and eleostearic acids, as well as those made from partial esters of stearic acid.

The preparation of the class of compounds useful in the compositions of the invention can be further illustrated by the following specific example:

*Example I*

An acid ester of a dimeric unsaturated fatty acid and a partial fatty acid ester of an alkyl anhydride was prepared by admixture and reaction of 428 parts by weight of sorbitan monooleate (manufactured by the Atlas Powder Company of Wilmington, Delaware, and marketed under the name "Span 80") with 560 parts by weight of dimerized linoleic acid (manufactured by Emery Industries, Inc. of Cincinnati, Ohio, and marketed under the name of Emery 955 Dimer Acid). The reaction mixture was heated under reflux, until 18 parts by weight of water had been trapped off, the maximum temperature reached by the reaction mixture being 500° F. The dimerized linoleic acid of this example had the following characteristics:

|                         |                               |
|-------------------------|-------------------------------|
| Physical state          | Straw-colored viscous liquid. |
| Molecular weight        | 564 (approx.).                |
| Gravity, °API           | 13.0.                         |
| Viscosity, SUV, 200° F. | 597.                          |
| Flash, OC, °F.          | 510.                          |
| Fire, OC, °F.           | 575.                          |
| Color, NPA              | +10.                          |
| Iodine No., Mod. Hanus  | 83.3.                         |
| Saponification No.      | 186.                          |
| Neutralization No.      | 182.                          |
| Dimer content           | 85% (approx.).                |
| Trimer and higher       | 12% (approx.).                |
| Monomer                 | 3% (approx.).                 |

The properties of the sorbitan monooleate were as follows:

|                                      |                 |
|--------------------------------------|-----------------|
| Molecular weight                     | 428 (approx.).  |
| Gravity, °API                        | 10.1.           |
| Sp. gr., 60°/60° F                   | 0.999.          |
| Lb./gal., 60° F                      | 8.32.           |
| Viscosity, SUV:                      |                 |
| 100° F                               | 1827.           |
| 210° F                               | 108.3.          |
| Flash, P-M, °F                       | 400.            |
| Flash, OC, °F                        | 410.            |
| Fire, OC, °F                         | 450.            |
| Pour, °F                             | +10.            |
| Physical state, room temp            | Viscous liquid. |
| Color, ASTM union                    | 4.5.            |
| Water by dist'n, percent             | Nil.            |
| Carbon residue, Conradson, percent   | 2.94.           |
| Neutralization value, ASTM D974-51T, |                 |
| total acid No                        | 6.15.           |
| pH value, glass-calomel electrodes   | 7.0.            |
| Saponification No., ASTM D94-48T     | 149.0.          |
| Acetyl value, Gulf 433               | 142.            |
| Ash, percent                         | 0.212.          |

The product obtained in the above-described reaction was a clear, viscous liquid containing predominantly mono-acid esters of dimerized linoleic acid and sorbitan monooleate, having the following physical properties:

|    |                                      |                 |
|----|--------------------------------------|-----------------|
| 5  | Gravity, °API                        | 13.4.           |
|    | Sp. gr., 60°/60° F                   | 0.977.          |
|    | Lb./gal., 60° F                      | 8.13.           |
|    | Viscosity, SUV, sec.:                |                 |
| 10 | 100° F                               | 9936.           |
|    | 210° F                               | 498.            |
|    | Flash, P-M, °F                       | 425.            |
|    | Pour, °F                             | 0.              |
| 15 | Physical state, room temp            | Viscous liquid. |
|    | Color, ASTM union                    | 6.0.            |
|    | Neutralization value, ASTM D974-51T, |                 |
|    | total acid No                        | 70.             |
|    | pH value, glass-calomel electrodes   | 4.6.            |

The acid esters of other dimerized unsaturated fatty acids and other partial fatty acid esters of alkyl anhydrides are similarly prepared.

The amount of the acid ester employed in the compositions of the invention depends upon the amount of the fatty amine salt of isoamyl octyl acid phosphate which has been used. Satisfactory results have been obtained with weight ratios of acid phosphate to acid ester of 1:1 to 1:4. Based on the weight of the total composition when using these ratios, the amount of acid ester comprises about 0.005 to about 0.8 percent by weight of the total composition. In any event the acid ester is used in an amount sufficient to prevent the formation of a precipitate when the composition is contaminated with a small amount of water.

The lubricating oil compositions of this invention can contain other additive agents if desired to improve other specific properties without deleteriously affecting the beneficial properties of the compositions. For example, pour point depressors, viscosity and viscosity index improvers, dyes, sludge inhibitors and the like can be used. Also, if desired, the oil can contain a foam inhibitor such as organo-silicon oxide condensation products, organo-silic平 condensation products and the like.

The individual constituents of the compositions of this invention may be added to the lubricating oil base in any order or simultaneously, either per se or in the form of a mineral oil concentrate. The latter practice is sometimes desirable in order to facilitate compounding of the compositions.

To illustrate the improved properties of the compositions of the invention, separate samples of compositions contaminated with water were compared with the base oil and other compositions containing an acid ester. The base oil used in the test was a highly refined aluminum chloride treated paraffinic turbine oil stock having an API gravity between about 30.5° and 32.5° and a viscosity of about 150 SUS at 100° F. In each instance the oil also contained 0.0033 percent by weight of Dow-Corning silicone Fluid 200 as a foam inhibitor. In order to determine the stability of the compositions the separate samples were stored in the sunlight in glass containers for 20 days. At the end of the 20-day period, the samples were examined for precipitate and for haze.

The improved rust-inhibiting properties of the compositions of the invention have been demonstrated by subjecting the separate samples to the procedure of ASTM test D943-47T. Briefly, this test is carried out by passing oxygen at a measured rate of 3 liters per hour into an oil-water mixture maintained at 203° F. and having an iron coil immersed therein. According to the procedure followed herein, the test was carried out for 500 hours. The corrosion-inhibiting properties of the compositions were determined by examining the iron coil before and after completion of the test. The amount of rust on the coil was thus used to determine the effectiveness of the composition in preventing rust.

The results of the 20-day storage test and the ASTM D943-47T test are tabulated as follows:

| Composition, percent by wt.                                                           | A           | B           | C           | D           | E       |
|---------------------------------------------------------------------------------------|-------------|-------------|-------------|-------------|---------|
| Base oil                                                                              | 100         | 100         | 98.63       | 98.63       | 98.86   |
| 2,6-di-tertiary-butyl-4-methylphenol                                                  |             |             | 1.25        | 1.25        | 1.0     |
| Zinc dihexyl thiophosphate                                                            |             |             | 0.1         | 0.1         | 0.1     |
| Cocoamine isoamyl octyl orthophosphate                                                |             |             | 0.012       | 0.012       | 0.016   |
| Dimerized linoleic acid-sorbitan monooleate acid ester reaction product of Example I. |             |             |             |             | 0.024   |
| Distilled water (added)                                                               |             | 0.5         |             | 0.5         | 0.5     |
| Inspection:                                                                           |             |             |             |             |         |
| Sunlight stability test (Mod.) after 20 days—                                         |             |             |             |             |         |
| Precipitate                                                                           | nil         | nil         | nil         | medium      | nil     |
| Haze                                                                                  | nil         | trace       | nil         | medium      | nil     |
| Amount of Rust, ASTM D943-47T, 500 Hours, Iron Coil                                   | heavy rust. | heavy rust. | light rust. | light rust. | bright. |

As can be noted from the data in the above table, the base oil gave satisfactory performance in the stability tests. Likewise the base oil containing 0.5 percent by weight of water was satisfactory. Even composition C passed the sunlight stability test when there was no water present. However, when 0.5 percent by weight of water was added to composition C the composition formed a medium amount of precipitate and haze after 20 days of exposure (composition D). It will be further noted, however, that when a small amount of the acid ester was employed, there was substantially no precipitate and no haze (composition E). Thus, as evidenced by composition E, the compositions of the invention resist the formation of precipitate and haze even when contaminated with water. As further evidenced from the data in the above table, the compositions of the invention in addition to having improved storage stability also give greater protection against rusting.

While the invention has been described above with reference to certain specific embodiments thereof by way of illustration, it is to be understood that the invention is not limited to such embodiments except as hereinafter defined in the appended claims.

We claim:

1. An improved turbine oil consisting essentially of a major proportion of a mineral lubricating oil and minor proportions consisting of about 0.1 to about 2.0 percent by weight of an alkyl phenol, said alkyl phenol containing at least one alkyl group containing between 3 and 12 carbon atoms, about 0.01 to about 0.1 percent by weight of a metal alkyl thiophosphate, said alkyl group containing between 3 and 12 carbon atoms, about 0.005 to about 0.2 percent by weight of a substantially neutral addition product of 3-methylbutyl,2-ethylhexyl acid orthophosphate and a primary fatty amine, said amine being a mono-alkyl amine containing from 8 to 18 carbon atoms, and about 0.005 to about 0.8 percent by weight of an acid ester of (1) a dimeric acid derived from an unsaturated fatty acid containing from 6 to 22 carbon atoms and having from 2 to 3 ethylenic linkages per molecule and (2) a partial ester of a fatty acid containing from 12 to 24 carbon atoms and an alitol anhydride, said acid ester containing at least one unreacted carboxyl group per molecule.

2. An improved turbine oil consisting essentially of a major proportion of a mineral lubricating oil and minor proportions consisting of about 0.1 to about 2.0 percent by weight of an alkyl phenol, said alkyl phenol containing at least one alkyl group containing between 3 and 12 carbon atoms, about 0.01 to about 0.1 percent by weight of a metal alkyl thiophosphate, said metal being a metal of group II of the periodic system and said alkyl thiophosphate containing at least one alkyl group containing between 3 and 12 carbon atoms, about 0.005 to about 0.2 percent by weight of the cocoamine salt of 3-methylbutyl,2-ethylhexyl acid orthophosphate, and an acid ester of a dimer of linoleic acid and sorbitan monooleate, said acid ester containing at least one unreacted carboxyl group per molecule and wherein the weight ratio of the cocoamine salt of 3-methylbutyl,2-ethylhexyl acid orthophosphate to said acid ester is between about 1:1 and 1:4.

8  
having from 2 to 3 ethylenic linkages per molecule and (2) a partial ester of a fatty acid containing 18 carbon

atoms and a hexitol anhydride, said acid ester containing at least one unreacted carboxyl group per molecule.

3. An improved turbine oil consisting essentially of a major proportion of a mineral lubricating oil and minor proportions consisting of about 0.1 to about 2.0 percent by weight of a tertiary alkyl phenol, said tertiary alkyl phenol containing at least one alkyl group containing between 3 and 12 carbon atoms, about 0.01 to about 0.1 percent by weight of a metal alkyl thiophosphate, said metal being a metal of group II of the periodic system and said alkyl thiophosphate containing at least one alkyl group containing between 3 and 12 carbon atoms, about 0.005 to about 0.2 percent by weight of the cocoamine salt of 3-methylbutyl,2-ethylhexyl acid orthophosphate, and about 0.005 to about 0.8 percent by weight of an acid ester of a dimer of linoleic acid and sorbitan monooleate, said acid ester containing at least one unreacted carboxyl group per molecule.

4. An improved turbine oil consisting essentially of a major proportion of a mineral lubricating oil and minor proportions consisting of about 0.1 to about 2.0 percent by weight of a tertiary alkyl phenol, said tertiary alkyl phenol containing at least one alkyl group containing between 3 and 12 carbon atoms, about 0.01 to about 0.1 percent by weight of a metal alkyl thiophosphate, said metal being a metal of group II of the periodic system and said alkyl thiophosphate containing at least one alkyl group containing between 3 and 12 carbon atoms, about 0.005 to about 0.2 percent by weight of the cocoamine salt of 3-methylbutyl,2-ethylhexyl acid orthophosphate, and an acid ester of a dimer of linoleic acid and sorbitan monooleate, said acid ester containing at least one unreacted carboxyl group per molecule and wherein said acid ester is present in an amount sufficient to prevent the formation of a precipitate when said turbine oil is contaminated with water.

5. An improved turbine oil consisting essentially of a major proportion of a mineral lubricating oil and minor proportions consisting of about 0.1 to about 2.0 percent by weight of a tertiary alkyl phenol, said tertiary alkyl phenol containing at least one alkyl group containing between 3 and 12 carbon atoms, about 0.01 to about 0.1 percent by weight of a metal alkyl thiophosphate, said metal being a metal of group II of the periodic system and said alkyl thiophosphate containing at least one alkyl group containing between 3 and 12 carbon atoms, about 0.005 to about 0.2 percent by weight of the cocoamine salt of 3-methylbutyl,2-ethylhexyl acid orthophosphate, and an acid ester of a dimer of linoleic acid and sorbitan monooleate, said acid ester containing at least one unreacted carboxyl group per molecule and wherein the weight ratio of the cocoamine salt of 3-methylbutyl,2-ethylhexyl acid orthophosphate to said acid ester is between about 1:1 and 1:4.

6. An improved turbine oil consisting essentially of a major proportion of a mineral lubricating oil and minor proportions consisting of about 0.1 to about 2.0 percent by weight of a tertiary alkyl phenol, said tertiary alkyl phenol containing at least one alkyl group containing

between 3 and 12 carbon atoms, about 0.01 to about 0.1 percent by weight of a metal di-alkyl thiophosphate, said metal being a metal of group II of the periodic system and said di-alkyl thiophosphate containing at least one alkyl group containing between 3 and 12 carbon atoms, about 0.005 to about 0.2 percent by weight of the cocoamine salt of 3-methylbutyl,2-ethylhexyl acid orthophosphate, and an acid ester of a dimer of linoleic acid and sorbitan monooleate, said acid ester containing at least one unreacted carboxyl group per molecule and wherein the weight ratio of the cocoamine salt of 3-methylbutyl,2-ethylhexyl acid orthophosphate to said acid ester is between about 1:1 and 1:4.

7. An improved turbine oil consisting essentially of a major proportion of a mineral lubricating oil and minor proportions consisting of about 0.1 to about 2.0 percent by weight of a tertiary butyl cresol, about 0.01 to about 0.1 percent by weight of a metal di-alkyl thiophosphate, said metal being a metal of group II of the periodic system and said di-alkyl thiophosphate containing at least one alkyl group containing between 3 and 12 carbon atoms, about 0.005 to about 0.2 percent by weight of the cocoamine salt of 3-methylbutyl,2-ethylhexyl acid orthophosphate, and an acid ester of a dimer of linoleic acid and sorbitan monooleate, said acid ester containing

at least one unreacted carboxyl group per molecule and wherein the weight ratio of the cocoamine salt of 3-methylbutyl,2-ethylhexyl acid orthophosphate to said acid ester is between about 1:1 and 1:4.

- 5 8. An improved turbine oil consisting essentially of a major proportion of a mineral lubricating oil and minor proportions consisting of about 0.1 to about 2.0 percent by weight of 2,6-di-tertiary-butyl-4-methylphenol, about 0.01 to about 0.1 percent by weight of zinc dihexyl thiophosphate, about 0.005 to about 0.2 percent by weight of the cocoamine salt of 3-methylbutyl,2-ethylhexyl acid orthophosphate, and about 0.005 to about 0.8 percent by weight of an acid ester of a dimer of linoleic acid and sorbitan monooleate, said acid ester containing at least one unreacted carboxyl group per molecule.
- 10

References Cited in the file of this patent

UNITED STATES PATENTS

- |    |           |              |               |
|----|-----------|--------------|---------------|
| 20 | 2,364,283 | Freuler      | Dec. 5, 1944  |
|    | 2,371,655 | Smith et al. | Mar. 20, 1945 |
|    | 2,631,979 | McDermott    | Mar. 17, 1953 |

FOREIGN PATENTS

- |    |         |               |              |
|----|---------|---------------|--------------|
| 25 | 428,864 | Great Britain | May 15, 1935 |
|----|---------|---------------|--------------|